

## UNITED STATES PATENT OFFICE

2,191,803

## ABRASIVE MATERIAL

Frank D. Oesterle, Teaneck, N. J., and George Zellar, Harrison, N. Y., assignors to Western Electric Company, Incorporated, New York, N. Y., a corporation of New York

No Drawing. Application July 2, 1938,  
Serial No. 217,216

5 Claims. (Cl. 51—280)

This invention relates to an abrasive material and more particularly to an abrasive material peculiarly adapted for use in finishing and re-finishing ornamental surfaces.

5 There is a great variety of procedures whose purpose is to produce an ornamental appearance upon a surface by means of coatings applied thereto, coatings of paint, varnish, enamel, and the like, oils, waxes and pastes of many kinds, 10 platings of metal deposited by spraying, electrodeposition, chemical deposition, etc., and others in almost indefinite variety. In a great many instances of such procedures, an abrasive medium may be used to modify the original surface, the 15 surface of some intermediate coating thereon, or the final surface. Purpose of such abrasive may be to remove larger or smaller irregularities, to roughen or matt a surface to give anchorage to a coating to be applied thereto or to give a desired final matt appearance, or to smooth or 20 polish the surface.

To effect such abrasive results, it has long been well known to use powdered abrasives, sand, emery, carborundum and the like attached to a 25 laminar base, paper, cloth, felt, and such by means of common adhesives like glue, thus making the well known sand paper, emery cloth, carborundum boards, and such. These abrasive tools suffer from two familiar defects: they are 30 stiff generally, and the abrasive grains are rigidly secured by the adhesives commonly employed to the backing. Hence, in use, especially on a curved or warped surface, in some instances such abrasive sheets will not conform properly to the 35 surface and unless great care is exercised the abrading is uneven. If the abrasive sheet is forced to curve beyond its naturally limited ability, it may tend to crack and the grains along the sharply folded crack may form a saw edge which 40 may do difficultly repairable damage. Also, the grains are in effect miniature planing tools mounted by the rigid adhesive on the backing sheet which is itself rendered stiff and rigid by the absorbed or impregnating adhesive. Hence the 45 permissible pressure, to avoid too deep cutting, i. e., unsightly scratching, is limited by those of the grains which protrude beyond the average surface of the grains; and, because a few grains are therefore excessive in effect, the majority 50 must be inefficiently used.

An object of the present invention is to produce an abrasive material of the general nature described, which shall be highly efficient in use, durable, capable of acting under high pressure without producing objectionable scratching, and

well adapted to produce a uniform effect on curved and irregular surfaces.

With these and other objects in view, one embodiment of the invention may comprise a flexible base such as loosely woven or knitted textile fabric, a body thereon of flexible and resilient adhesive material, e. g., printers roller compound of glue and glycerine or soft rubber, and abrasive grains embedded therein.

Other objects and features of the invention will 10 clearly appear from the following detailed description of embodiments thereof.

To make one preferred embodiment of the invention, a sheet of ordinary commercial unbleached muslin may be used as the base, say a 15 muslin having 56 x 56 threads to the inch. For convenience of use, it is preferred to apply the adhesive compound to one side only of this cloth base, although both sides may be coated 20 if desired.

A preferred compound for use as the body coat on the cloth may have the following composition:

|                     | Per cent |
|---------------------|----------|
| Dry flake glue..... | about 60 |
| Glycerine.....      | about 30 |
| Water.....          | about 10 |

and for some purposes there may be added to the above about 3% of linseed oil which acts apparently to toughen the compound without 30 hardening it. To preserve this compound against attack by mold, or by flies and other insects, there may also be added enough of a saturated solution of copper sulfate in water to give the whole a content of about 0.1% copper sulfate. 35

The above formula yields a compound giving a product as described below which is eminently satisfactory for use in roughening and smoothing varnished, japanned, enameled or lacquered surfaces on sheet metal, especially where the 40 metal sheet has been formed into curved or warped contours.

The above described compound is one well known and commonly obtainable in commerce under the general name of "printer's roller compound", it being used widely in the printing art as material for making rollers used in apparatus for both direct and offset printing. 45

To apply the compound to the cloth or other base, the compound may be melted and made 50 sufficiently liquid to form a closely adherent coating on the cloth without at the same time saturating or penetrating the cloth completely. The compound may be applied to the cloth in any convenient and suitable manner, e. g., by running 55

the cloth over a roller which dips into the surface of the melted compound, or by painting the melted compound or pouring it and spreading it on the cloth.

5 The coated cloth may then be allowed to cool, dry and partially harden to still somewhat "tacky" surface state. Abrasive powder is then applied to the faintly sticky or tacky surface of the compound and the whole allowed to cool and 10 harden completely.

15 A preferred abrasive for use as described above on lacquered metal or the like, is artificial aluminum oxide, such for example as that commercially known by the trade name "Aloxite", 20 with a grain size of 120 mesh. It may be applied to the tacky adhesive on the cloth by any suitable and convenient method, e. g., by sprinkling an excess on and shaking, or by passing the 25 coated cloth in front of a dust blower charged with the abrasive, or by passing the coated cloth over a roller located in a container filled with the abrasive.

30 The coated cloth thus loosely charged with abrasive is then preferably passed between rollers to embed the abrasive firmly in the resilient jelly-like layer of adhesive. Because of the jelly consistency and character of the resilient coating this is not ordinarily to be accomplished by pressure alone. Preferably the roller against 35 which the uncoated rear face of the cloth runs is cold, even chilled by being hollow and having cold water circulated through it, while the co-operating roller which runs against the abrasive and adhesive coated side is heated by any suitable and convenient means such as steam. The 40 heated roller is preferably maintained at such a temperature, dependent among other factors on the speed of the coated sheet over it and the thickness and intrinsic hardness of the adhesive used, as will superficially melt the upper surface of the adhesive to receive and partially embrace the grains of abrasive, but will not melt the under surface of the adhesive enough to cause it to soak through the cloth.

45 The laminar product, after being thus calendered, is then allowed to cool and harden completely and is then ready for use.

50 The product made as above described, with the glue-glycerine adhesive whose ingredient proportions are specified above and with 120 mesh Aloxite as its abrasive, may be compared, for 55 illustration of its advantages, with an ordinary sand paper or emery cloth having plain glue as adhesive and 240 mesh silica sand or emery as abrasive. The sand paper or emery cloth is stiff. It cannot be bent to any reasonably small radius without the production of saw edged, cracked creases which are practically certain to produce 60 unsightly scratching, especially if applied to concavely curved work. The product of the invention is nearly as flexible and crumplable as the original cloth. It creases in much the same manner as the original cloth, in creases or folds whose edges are not cracked, and hence not saw-toothed.

65 Although the product of the invention as described has an abrasive of 120 mesh, twice as coarse as the 240 mesh abrasive of the sand paper or emery cloth, it may be applied to and 70 rubbed over a piece of work under even greater pressure than that which causes the sand paper or emery cloth described to produce objectionable scratches, without any such objectionable effect.

75 Furthermore, the product of the invention may be used far longer before becoming useless

through clogging with abraded particles than a sand paper, emery cloth or the like of ordinary construction and of the same grain size.

It is suggested that the great difference in effectiveness between the product of the invention and comparable materials of the prior art is perhaps due to the fact that the abrasive grains, the 10 miniature planing tools, of the invention are resiliently mounted on the laminar base by the 15 resilient adhesive, so that any grain that projects beyond the average level of the cutting points of the grains generally is relatively easily forced back into the resilient jelly until the cutting pressure is fairly evenly divided among all the grains. In a sand paper, emery cloth or the 20 like made in the ordinary fashion with a hard adhesive, the grains are rigidly held relatively to each other and to the backing. Hence any grains protruding beyond the average will not yield and retire, but will bear all the burden of 25 the pressure in its neighborhood and so cut abnormally deeply until it has entered the work far enough to permit nearby grains to begin to cut.

30 The flexibility of the product of the invention arises primarily from the resilient, jelly-like nature of the adhesive. Hence even if the cloth, paper or other backing be saturated or coated with the adhesive on both sides and provided with abrasive on both sides, the flexibility and softness of the double sided product are but little less 35 than in the one sided product, and are still far greater than with a hard adhesive such as glue.

35 In another method of making the product of the invention, the adhesive compound may be prepared and melted as before, and when melted may be charged with the powdered abrasive by stirring the latter into the melted abrasive until evenly distributed therethrough. This mixture of adhesive and abrasive may then be coated upon a suitable base or backing in any suitable manner.

40 The invention is not limited to the use of a laminar backing or even to a flexible backing. Thus in the "rifles" used as sharpening instruments for scythes, sickles and the like in place 45 of whetstones and which comprise a rigid core, e. g., of wood, ordinarily of a generally oval or elliptical cross section, and covered with an abrasive such as powdered emery secured thereto with glue or other ordinarily rigid and hard adhesive, a considerable improvement in useful life may be attained by the use of a resilient, 50 jelly-like adhesive. Such rifles, glaze and become ineffective through clogging between the cutting grains with particles of metal. Where the grains are rigidly held by the adhesive, the particles are readily and rapidly held and jammed between the grains. Where the grains, however, have a 55 resilient freedom of motion relatively to each other, material jammed and caught between the grains during one working stroke of the rifle are apt to be released and shaken out at the next.

60 Where even more resilience is desired, e. g., in working on a corrugated or other analogous surface, a resilient wad-like or pad-like backing or base may be used. Thus in another embodiment of the invention a wad or mass of fibrous material, such as oakum or waste, may be more or less saturated with the adhesive in a molten state, partially hardened, rolled in the powdered 65 abrasive, and completely hardened. Or, if the abrasive be incorporated into the compound as already described, such a wad or mass of oakum, waste or the like may be worked in the molten 70 abrasive charged compound until saturated.

through and then cooled and hardened. Such a mass will then present fresh working surfaces wherever torn or cut apart. For such embodiments of the invention resiliently spongy masses 5 may be used as a base, e. g., natural sponge, sponge rubber, or the like.

While in the adhesive compound described above the glue and glycerine are given in the ratio of two to one (60% to 30%), this proportion 10 of these two ingredients may be varied from about one to one (45% to 45%) to about five to one (75% to 15%) if it be desired to vary the hardness and toughness of the compound without taking away its resilient character. So also, 15 the water content, given above as 10%, may be varied relatively to the total amount of glue and glycerine combined. The embodiments disclosed are illustrative and may be varied in many ways without departing from the spirit and scope 20 of the invention as pointed out in and limited solely by the appended claims.

What is claimed is:

1. In a material for abrasive uses comprising a limply flexible base of textile threads and a 25 granular abrasive of hard mineral substance, an adhesive compound to secure the abrasive to the base and comprising 45 parts to 75 parts dry glue and 45 parts to 15 parts glycerine and 5 parts to 15 parts water and 1 part to 5 parts linseed oil. 30 2. In a material for abrasive uses comprising a limply flexible base of textile threads and a

granular abrasive of hard mineral substance, an adhesive compound to secure the abrasive to the base and comprising 45 parts to 75 parts dry glue and 45 parts to 15 parts glycerine and 5 parts to 15 parts water and 1 part to 5 parts linseed oil 5 and  $\frac{1}{20}$  to  $\frac{1}{4}$  part copper sulfate.

3. In a material for abrasive uses comprising a limply flexible base of textile threads and a 10 granular abrasive of hard mineral substance, an adhesive compound to secure the abrasive to the base and comprising about 60 parts dry glue and about 30 parts glycerine and about 10 parts water and about 3 parts linseed oil.

4. In a material for abrasive uses comprising a limply flexible base of textile threads and a 15 granular abrasive of hard mineral substance, an adhesive compound to secure the abrasive to the base and comprising about 60 parts dry glue and about 30 parts glycerine and about 10 parts water and about 3 parts linseed oil and about 20  $\frac{1}{16}$  part copper sulfate.

5. In a material for abrasive uses comprising a limply flexible base of textile threads and a 25 granular abrasive of hard mineral substance, an adhesive compound to secure the abrasive to the base and comprising 60 parts dry glue and 30 parts glycerine and 10 parts water and 3 parts linseed oil.

FRANK D. OESTERLE.  
GEORGE ZELLAR.